

## UNITED STATES PATENT OFFICE

2,548,494

## ESTERS OF TRIMETHYLAIDIPIC ACID

Paul V. Smith, Jr., Westfield, N. J., assignor to  
Standard Oil Development Company, a corpora-  
tion of Delaware

No Drawing. Application August 3, 1948,  
Serial No. 42,335

7 Claims. (Cl. 260—485)

1

This invention relates to a new class of com-  
pounds which have been found to be particularly  
suitable for use as synthetic lubricants.

In the lubricant art, considerable progress has  
been realized in recent years in the production  
of lubricants characterized by one or more spe-  
cific properties and adapted for particular uses.  
In the main, this progress can be attributed to  
two developments: the first, new refining pro-  
cedures, and the second, addition agents capable  
of imparting particular properties to available  
lubricants. Thus, viscosity index improvers and  
pour depressants are added to automotive lubri-  
cants to render the lubricants more adaptable to  
wide changes in temperature conditions, while  
other agents are added to improve the load carry-  
ing properties of a lubricant which is to be em-  
ployed, for example, under extreme pressure con-  
ditions.

Recently, in an effort to obtain superior lubri-  
cants endowed with specific and superior char-  
acteristics, a new field has been explored, namely,  
the synthesis of lubricants from various materials.  
Esters represent one class of materials  
which have attracted unusual interest as syn-  
thetic lubricants. In general, they are character-  
ized by higher viscosity indices and lower pour  
point than mineral oils of corresponding viscosity.  
The esters described in the present specification  
have been found to exhibit these desirable prop-  
erties. Lubricants possessing such properties are  
of special value in the lubrication of engines  
which are subjected to high temperatures such  
as combustion turbine engines, particularly those  
of the "prop-jet" type. Mineral oil lubricants  
containing added viscosity index improvers,  
thickeners or other highly non-volatile additives  
are undesirable for use in such engines because  
of the tendency to leave a residue which accumu-  
lates and interferes with the operation of the  
engine. A synthetic lubricant of the type de-  
scribed in the present specification is especially  
adapted to use under such conditions, since the  
lubricant contains no additives and thus tends  
to leave no residue upon volatilization.

The new compounds of the present invention  
which constitute a class of esters which have  
been found to possess properties indicating their  
usefulness as synthetic lubricating oils are fully  
esterified trimethyladipic acids, the acids having  
been esterified by monohydric alcohols which  
contain oxygen or sulfur atoms in ether or thio-  
ether linkages. The ester groups which replace  
the hydrogen atoms of the two carboxyl groups of  
the acid contain straight chain or branched chain

2

hydrocarbon groups and may be alike or unlike  
in chain length or other characteristics.

Trimethyladipic acid, which undoubtedly con-  
sists of a mixture of two isomeric forms having  
5 the structures



10 and



15

may be readily prepared by oxidizing dihydroiso-  
phorone with nitric acid, a detailed method for  
carrying out the preparation being described  
hereinafter. The trimethyladipic acid may be

20 readily esterified by refluxing with a suitable  
alcohol or mixture of alcohols in the presence  
of a catalyst such as p-toluenesulfonic acid  
monohydrate and a suitable medium for entrain-  
ing water during the reaction.

25 The monohydric alcohols which may be em-  
ployed in preparing the trimethyladipic acid  
esters of the present invention are aliphatic  
alcohols of the general formula

30

$\text{RXR}'\text{OH}$

where R is (1) an alkyl group of 1 to 18 carbon  
atoms, or (2) an organic group consisting of a  
series of saturated aliphatic hydrocarbon radi-  
35 cals interlinked by oxygen or sulfur atoms or  
both, the number of oxygen and sulfur atoms  
not exceeding 5, and the total number of carbon,  
oxygen and/or sulfur atoms being from 4 to 18,  
with the provision that there are at least two  
40 carbon atoms between each pair of oxygen or  
sulfur atoms and between the atom X and the  
first oxygen or sulfur atom; X is oxygen or sulfur;  
and R' is a saturated aliphatic hydrocarbon  
group of 2 to 3 carbon atoms, alcohols in which

45 R' represents the group  $-\text{CH}_2\text{CH}_2-$  being gener-  
ally preferred. The total number of carbon,  
oxygen and/or sulfur atoms in the two alcohol  
residues attached to the acid radical should be  
at least 12.

50 Among the ether-alcohols and thioether-alco-  
hols which have been found to be particularly  
suitable for use as esterifying alcohols in the  
preparation of the compounds of the present  
invention may be mentioned the following, it

55 being understood that these are illustrative only

and that the invention is not to be considered as limited to the use of such compounds:

Ethylene glycol mono-n-butyl ether  
Ethylene glycol mono-2-ethylbutyl ether  
Ethylene glycol mono-2-ethylhexyl ether  
Ethylene glycol mono-tert.-octyl ether  
 $\beta$ -n-Butylmercaptoethanol  
 $\beta$ -tert.-octylmercaptoethanol  
 $\beta$ -n-Dodecylmercaptoethanol  
Diethylene glycol mono-n-butyl ether  
Diethylene glycol mono-2-ethylbutyl ether  
Diethylene glycol mono-2-ethylhexyl ether  
Propylene glycol mono-butyl thioether  
Propylene glycol mono-tert.-octyl thioether  
Propylene glycol mono-n-dodecyl thioether  
n-Butylmercaptoethoxyethanol  
Tert.-octylmercaptoethoxyethanol  
n-Dodecylmercaptoethoxyethanol

prepared by esterifying the trimethyladipic acid obtained in the above described process in accordance with the following procedure: A mixture containing 1 mol of trimethyladipic acid, 5 2.2 mols of alcohol, 0.7% by weight of p-toluenesulfonic acid monohydrate, and a water entraining material such as benzene, toluene, naphtha or the like was refluxed until no more water collected in the water trap connected to the refluxing condenser. Then the mixture was washed three times with a saturated solution of sodium carbonate and once with water. After drying over a dessicant such as Drierite (anhydrous calcium sulfate) the product was stripped at 10 210-225° under 5 mm. pressure.

15 The esters obtained by the above typical reaction method were found to have the properties set forth in the table.

Table

| Alcohols Used in Esterification         | Kinematic Viscosity |         | ASTM Slope | Viscosity Index | ASTM Pour Point |
|-----------------------------------------|---------------------|---------|------------|-----------------|-----------------|
|                                         | 100° F.             | 210° F. |            |                 |                 |
| Butyl carbitol                          | 16.050              | 3.701   | 0.724      | 136             | °F.             |
| 2-Ethylhexyl carbitol                   | 17.640              | 3.987   | 0.711      | 145             | <-35            |
| Tripropylene glycol monoisopropyl ether | 170.000             | 18.130  | 0.618      | 118             | <-35            |
| $\beta$ -tert.-Octylmercaptoethanol     | 616.900             | 41.940  | 0.595      | 111             | -20             |
|                                         |                     |         |            |                 | 0               |

n-Butylmercaptopropoxypropanol  
Tert.-octylmercaptopropoxypropanol  
n-Dodecylmercaptopropoxypropanol  
Propylene glycol mono-n-butyl ether  
Dipropylene glycol monomethyl ether  
Dipropylene glycol monoethyl ether  
Dipropylene glycol mono-n-butyl ether  
Tripropylene glycol monomethyl ether  
Tripropylene glycol monoethyl ether  
Tripropylene glycol mono-n-butyl ether  
Propylene glycol monoisopropyl ether  
Dipropylene glycol monoisopropyl ether  
Tripropylene glycol monoisopropyl ether

Many of the above listed ether alcohols, formed 45 by the reaction of ethylene oxide or propylene oxide with aliphatic alcohols, are known in the industry as "Dowanol," "Cellulosolve," or "Carbitols."

Data will be given below showing properties 50 of four examples of esters of trimethyladipic acid which illustrate the present invention. All of these esters are prepared by esterifying trimethyladipic acid, the latter being prepared by the following method: In an all glass apparatus consisting of a 3-liter flask fitted with a stirrer, condenser and dropping funnel was placed 1.5 liters (16 mols) of 50% aqueous nitric acid solution. This material was heated to boiling and 350 g. (2.5 mols) of dihydroisophorone was added dropwise at such a rate that refluxing continued rapidly. The refluxing was continued for several hours after the addition of the dihydroisophorone was complete, after which the resulting solution was nearly neutralized with sodium hydroxide and the top layer resulting from this procedure separated. After washing this product three or four times with a saturated sodium chloride solution, about 100-200 cc. benzene was added and the water removed by azeotropic distillation. The solvent was then removed by vacuum stripping to give 307 g. of product. (The crude acid may be used as such or the material may be distilled.)

The esters described in the table below were 75

35 The above data indicate that the esters of trimethyladipic acid prepared from alcohols containing ether or thioether linkages contain characteristics with regard to viscosity index and pour point which indicate their suitability for general use as a lubricating oil, and particularly under conditions where the use of non-volatile additives is not desirable.

40 The esters of the present invention not only possess good lubricating qualities in themselves, but they may be blended with mineral lubricating oils to give lubricants of improved viscosity index and pour point.

What is claimed is:

1. As a new composition of matter a fully esterified trimethyladipic acid, formed by esterifying trimethyladipic acid with at least one mono-hydric aliphatic alcohol of the general formula



where R is a member of the class consisting of (1) alkyl groups containing 1 to 18 carbon atoms each, and (2) organic groups each consisting of a series of aliphatic hydrocarbon radicals inter-linked by non-carbon atoms selected from the group consisting of oxygen and sulfur, the number of said non-carbon atoms not exceeding 5 and the total number of carbon atoms and said non-carbon atoms in radical R being from 4 to 18, wherein there are at least two carbon atoms between each pair of said non-carbon atoms and between the atom X and the first such non-carbon atom; X is an element of the group consisting of oxygen and sulfur; and R' is a saturated aliphatic hydrocarbon group of 2 to 3 carbon atoms; the total number of carbon and said non-carbon atoms in the two RXR'—groups attached to the acid radical being at least 12.

2. A composition according to claim 1 in which X of the formula is oxygen.

3. A composition according to claim 1 in which X of the formula is oxygen and in which all of the interlinking non-carbon atoms in radical R are oxygen atoms.

4. A composition according to claim 3 in which the radical R' is the group —CH<sub>2</sub>CH<sub>2</sub>—.
5. A composition according to claim 1 in which the esterifying alcohol is butyl carbitol.
6. A composition according to claim 1 in which the esterifying alcohol is 2-ethylhexyl carbitol.
7. A composition according to claim 1 in which the esterifying alcohol is tripropylene glycol monoisopropyl ether.

PAUL V. SMITH, JR.

## REFERENCES CITED

The following references are of record in the file of this patent:

## UNITED STATES PATENTS

| Number    | Name  | Date          |
|-----------|-------|---------------|
| 2,448,259 | Finch | Aug. 31, 1948 |

## OTHER REFERENCES

10 Beilstein: "Handbuch der organischen Chemie," 4th ed., vol. 2, page 715 (1920).